

# UNITED STATES PATENT OFFICE.

FRANZ THOMAS, OF SCHMÖLLN, GERMANY.

## PROCESS FOR FORMING CASEIN MASSES.

1,159,878.

Specification of Letters Patent.

Patented Nov. 9, 1915.

No Drawing.

Application filed December 5, 1912. Serial No. 735,113.

To all whom it may concern:

Be it known that I, FRANZ THOMAS, chemist, subject of the German Emperor, residing at 5 Amtsplatz, Schmölln, Duchy of Saxonia-Altenburg, German Empire, have invented a new and useful Improvement in Processes for Forming Casein Masses; and I do hereby declare the following to be a full, clear, and exact description of the same.

10 This invention relates to a process for forming casein masses, that is to say for producing from a supply of the liquids that are to be dealt with, such as solutions or suspensions of alkali caseinates, solid pieces or articles of the requisite size.

15 The invention has for its object to produce in the process of forming such solid pieces or articles certain desirable visual effects such as veining, graining, stratification designs, or the like, the process comprising a method of pouring or dropping portions of the liquid.

20 Heretofore it has not been found possible to produce figured or patterned articles of casein showing veins, graining or the like, by pouring. It was also quite impossible, by existing methods of producing colored masses of casein by pressing or rolling, to get the colors distributed in circles, a streaky 25 effect being obtained. In imitating horn, and particularly for making buttons, however, it is specially important to be able to obtain the colors in rings, because the material then resembles the natural horn, or the 30 like, more closely than the streaky colored effects heretofore obtainable.

35 I have discovered that figured varicolored casein masses can be produced by pouring variously colored or shaded solutions or suspensions of alkali caseinates on the surface of a solution of formaldehyde and an alkaline earth salt. A number of differently colored streams of the alkali caseinates solutions may be poured into the precipitation 40 bath at the same time without the streams becoming completely intermingled even when they enter the precipitation bath simultaneously. It might have been expected that complete admixture would ensue, accompanied by a uniform coloration devoid of figuring; but as a matter of fact this is not the case.

45 The method can be carried out in the following manner: In order to obtain annular 50 figurings or graining, the various colored solutions of alkali caseinates are allowed to

enter the precipitation bath in varying succession. I may use a solution of 1 kilogram of precipitated casein in 3 liters of an aqueous solution of sodium hydroxid containing 60 per liter 10 grams sodium hydroxid and cause the said solution to drop into a solution of 5 kilograms calcium chlorid in 100 liters water mixed with 5 liters of 40 per cent. formaldehyde. To the solution of casein I 65 may add according to the desired shade black colors for instance nigrosin or Chinese black, white colors, for instance chalk, gypsum, yellow colors for instance ocher, red colors for instance bole, etc. According to 70 the rate at which the streams of different colors are used the rings are obtained of smaller or greater width. It might be expected that the second drop introduced, after the first one, into the bath, would simply envelop the 75 first one, so that no figuring would subsequently be apparent in the slab or piece; as a fact however, the result is quite different, a hemispherical hollow being formed so that the further supply of material enters 80 the cavity first produced. The various strata also diffuse to some extent, so that delicate veinings or graining effects, such as are otherwise found only in natural products, ensue.

85 An alternative method of producing figured designs by pouring consists in allowing the differently colored caseinates solutions to enter the precipitating liquid simultaneously instead of successively. The differently colored solutions of casein are led into a common terminal nozzle from which they can be directed simultaneously on to the same point of the precipitation bath and thus form the same center. The solutions 90 can be maintained more or less separate by modifying their relative viscosity, thus producing either quite distinct or diffused effects.

95 I claim:

100 1. The process for the formation of spherical varicolored casein masses which consists in causing separate streams of variously colored or shaded solutions of alkali caseinate to fall freely vertically in the form of drops 105 on to a common point within a liquid precipitation bath, consisting of a solution of alkaline earth salt.

110 2. The process for the formation of spherical varicolored casein masses which consists in causing separate streams of variously colored or shaded solutions of alkali caseinate

having a different grade of viscosity to fall freely vertically in the form of drops on to a common point within a liquid precipitation bath, consisting of a solution of alkaline 5 earth salt.

3. The process for the formation of spherical varicolored casein masses which consists in causing separate streams of variously colored or shaded solutions of alkali caseinate

to fall freely vertically in the form of drops 10 on to a common point within a liquid bath of formaldehyde and alkaline earth salt.

In testimony whereof I affix my signature in presence of two witnesses.

FRANZ THOMAS.

Witnesses:

CHARLES NEUER,  
M. MÜLLER.